

## 1

3,238,166

PROCESS FOR ENDOWING PERMANENT DIRT-  
PREVENTING PROPERTY AND HARDNESS TO  
FABRICS OF SYNTHETIC FIBERS, AND RESIN  
COMPOSITION THEREFOR

Eiichi Kawai, Takatsuki-shi, Tadao Matsumoto, Toyonaka-shi, and Shigeru Tajima, Ashiya-shi, Japan, assignors to Sumitomo Chemical Company, Ltd., Osaka, Japan, a corporation of Japan

No Drawing. Filed Oct. 8, 1962, Ser. No. 229,171  
Claims priority, application Japan, Oct. 10, 1961,

36/36,747

4 Claims. (Cl. 260—29.4)

This invention relates to a process for imparting permanent and excellent hardness and soil resistance to fabrics of synthetic, hydrophobic fibers, particularly fabrics of polyester, polyacrylic, or partially acetylated cellulose fiber, or mixed spun fabrics thereof with cellulose or animal fibers, and to a resin composition therefor.

More particularly, the present invention relates to a process for imparting permanent soil resistance and hardness to fabrics as mentioned above, by soaking the same in a resin bath containing an aqueous solution of a vinyl polymer containing hydroxyl and aldehyde groups in the molecule which is obtained by saponification of a copolymer of vinyl acetate with acrolein or acrolein di-

15

20 25

At present, fabrics of synthetic fibers are widely utilized as clothing because of their ease of washing and their excellent wrinkle- or crease-resistance. However, the most significant drawbacks of such fabrics reside in that it is difficult to control the handling of fabric and that dirts tend to be adsorbed. Because of their ease of washing, which is one of the characteristics of the fabrics of synthetic fibers, they have been utilized mainly for those clothings which are laundered repeatedly, such as white shirts, blouses and sport shirts. Therefore, an indispensable requirement for synthetic fabric involves permanent improvement in handling and dirt-resistance. These improvements have been sought by those in the trade. Regarding polyamide and polyvinyl fiber fabrics, such improvements have recently been almost achieved. Regarding polyester, polyacrylic and partially acetylated cellulosic fiber fabrics, however, no satisfactory improvement has yet been obtained.

That is to say, fabrics of polyamide and polyvinyl fibers, have been treated, as in the case of cellulose fiber fabrics, with aminoplast, particularly with melamine resin, to obtain a durable, strong hardness. Polyester, polyacrylic and partially acetylated cellulosic fiber fabrics, however, have less affinity to such resins, hence, it is difficult to obtain permanent hardness by bondage of such resins, as shown in Table 1.

TABLE 1.—EFFECTS OF HARDENING AGENTS TO VARIOUS FABRICS<sup>1</sup>

|                                                             | Non-treated    |                            | Treated with a highly condensed urea-formaldehyde resin <sup>2</sup> |               | Treated with a methylated trimethylol-melamine <sup>3</sup> |               | Treated with P.V.A. <sup>4</sup> |               |
|-------------------------------------------------------------|----------------|----------------------------|----------------------------------------------------------------------|---------------|-------------------------------------------------------------|---------------|----------------------------------|---------------|
|                                                             | Before washing | After washing <sup>5</sup> | Before washing                                                       | After washing | Before washing                                              | After washing | Before washing                   | After washing |
| 40's cotton broad cloth                                     | 88             | 78                         | 115                                                                  | 105           | 90                                                          | 88            | 132                              | 87            |
| Sheer nylon                                                 | 57             | 55                         | 89                                                                   | 80            | 107                                                         | 103           | 87                               | 60            |
| Sheer polyethylene terephthalate                            | 77             | 81                         | 101                                                                  | 86            | 129                                                         | 91            | 102                              | 83            |
| Polyacrylonitrile fiber fabric muslin                       | 45             | 46                         | 75                                                                   | 53            | 98                                                          | 68            | 80                               | 50            |
| Partially after-acetylated cellulosic-fiber fabric tropical | 66             | 60                         | 125                                                                  | 65            | 153                                                         | 90            | 110                              | 60            |

<sup>1</sup> The effect of each hardening agent is determined by measuring the bending lengths and summing up the values of warp and weft directions (mm.). (CCC-T-191b method No. 5206).

<sup>2</sup> The resin was applied to the respective fabrics according to the following recipe:

A highly condensed urea-formaldehyde resin—10 g. Accelerator ACX (2-amino-2-methylpropanol hydrochloride)—1 g. Total amount was made 100 cc. by addition of water.

<sup>3</sup> The methylated trimethylolmelamine was applied to the respective fabrics according to the following recipe:

A methylated trimethylol amine—10 g. Accelerator ACX—1 g. Total amount was made 100 cc. by addition of water.

<sup>4</sup> P.V.A. is a 2% aqueous solution of polyvinyl alcohol.

<sup>5</sup> Respective washing was repeated 5 times by home-washing machine.

acetate, said aqueous solution being added with magnesium chloride as catalyst, and then subjecting the fabrics to conventional resin processing procedures such as preliminary drying, curing, soaking, etc.

Further, the present invention relates to a process for imparting more permanent soil resistance and hardness to such fabrics, by carrying out the above-mentioned process by combined use of at least one of other processing resin, such as dimethylolethyleneurea, dimethylolurone, dimethylolglyoxalmonourea, tetramethylolacetylenedurea, dimethyloltriazone, and their alkylated compounds.

55 The present inventors have found, through broad researches on resins capable of yielding an excellent hardening effect to polyester, polyacrylonitrile and partially acetylated cellulosic fiber fabrics, that such effect is easily obtained by employing a water soluble vinyl polymer containing hydroxyl and aldehyde groups in the molecule which is obtained by saponifying a copolymer of vinyl acetate with acrolein or with acrolein diacetate, said aqueous solution being added with magnesium chloride as catalyst.

60 Methods for producing the above-mentioned water-soluble vinyl polymer are well known from the description

in United States Patent Nos. 2,569,932, 2,485,239 and 2,657,192. Also, these patents describe that said water soluble vinyl polymer may be employed as an adhesive for cellophanes, paper or clothes or a sizing agent for nylon fabrics. However, there was no disclosure that such vinyl polymer can advantageously be utilized in imparting permanent hardness and soil resistance effect to specific textile fabrics.

Moreover, catalyst employed in the aforesaid patents are maleic acid, glycolic acid and others. The present inventors, however, discovered after minute studies to find out a catalyst effective in applying said water soluble vinyl polymer to polyester, polyacrylonitrile and partially acetylated cellulosic fiber fabrics, that magnesium chloride can give surprisingly significant hardness and soil resistance compared with other catalysts.

Table 2 shows the hardening effect obtained by using in combination with various catalyst a vinyl polymer "resin A," prepared in accordance with the example described later.

The water soluble vinyl polymers employed in the present invention are those having the structure

5



obtained, as mentioned before, by saponifying a copolymer of vinyl acetate with acrolein or acrolein diacetate, wherein X and Y are respectively whole numbers, and the ratio of X:Y is 5-20:95-80.

10

Thus, the vinyl polymers particularly suitable to accomplish the object of the present invention are those containing acrolein units in an amount between about 5 and 20 mol percent, ordinarily about 10 mol percent, on the basis of the vinyl polymer.

15

Also, the vinyl polymers employed may be any of those having a molecular weight of more than about 20,000 and less than about 1,000,000, and being water soluble. In case vinyl polymers having a molecular weight of less

20

TABLE 2.—HARDENING EFFECT OBTAINED BY TREATING PARTIALLY ACETYLATED CELLULOSIC FIBER FABRICS WITH A VINYL POLYMER "RESIN A" OF THE EXAMPLE IN COMBINATION WITH CATALYSTS. (BEND LENGTH, MM.)

| Catalyst            | Nontreated cloth | Maleic acid | $(\text{NH}_4)_2\text{HPO}_4$ | 2-amino-2-methyl propanol hydrochloride | $\text{Zn}(\text{NO}_3)_2$ | $\text{MgCl}_2$ | $\text{MgCl}_2 +$<br>dimethyloluron |
|---------------------|------------------|-------------|-------------------------------|-----------------------------------------|----------------------------|-----------------|-------------------------------------|
| Beforewash ing----- | 62               | 92          | 90                            | 98                                      | 93                         | 114             | 120                                 |
| After washing-----  | 55               | 71          | 68                            | 81                                      | 77                         | 100             | 112                                 |

An object of the invention is to provide a novel process for imparting permanent soil resistance and hardness to fabrics of synthetic fibers, especially to fabrics of polyester, polyacrylic, and partially acetylated cellulose fibers, of which the improvement as shown above has not yet been attained. Another object of the invention is to provide a resin composition used for the processing as above-mentioned. Other objects would be apparent as the description proceeds.

Accordingly, the present invention provides a resin composition used for the processing of fabrics of hydrophobic fibers to endow them with permanent soil resistance and hardness, which comprises an aqueous solution of a vinyl polymer composed of vinyl alcohol and acrolein units, said aqueous solution containing magnesium chloride as catalyst. Further, the invention provides a process for imparting permanent soil resistance and hardness to fabrics of hydrophobic fibers, which comprises soaking a fabric of a hydrophobic fiber in a resin bath containing an aqueous solution of a vinyl polymer composed of vinyl alcohol and acrolein units, said aqueous solution containing magnesium chloride as catalyst. More particularly, the present invention provides a process for imparting permanent soil resistance and hardness to fabrics of synthetic, hydrophobic fibers, which comprises soaking a fabric containing at least partially a fiber of the group of polyester, polyacrylonitrile and partially acetylated cellulose fibers, in a resin bath containing an aqueous solution of a vinyl polymer containing hydroxyl and aldehyde groups in the molecule which is obtained by saponification of a copolymer of vinyl acetate with a member selected from the group consisting of acrolein or acrolein diacetate, said aqueous solution being added with magnesium chloride as catalyst.

Furthermore, the present invention provides a process for imparting permanent soil resistance and hardness to such fabrics, which comprises soaking the fabric in a resin bath containing an aqueous solution of such vinyl polymer and an aminoplast, said aqueous solution being added with magnesium chloride as catalyst.

than such limitation are employed, the desired object of the present invention is hardly achieved.

40

Preferable magnesium chloride catalyst for the purpose of the present invention is prepared, for example, by adding more than about 15% of an aqueous 30% magnesium chloride solution to a 15% paste of said vinyl polymer.

45

The aminoplasts used in combination with the vinyl polymer for further increasing the permanent hardening and soil resistance are one or more of urea resins such as dimethylolurea, dimethylolethyleneurea, dimethyloluron, dimethylolglyoxalmonourein, tetramethylolacetylene-diurea, dimethyloltriazone and their alkylated derivatives. The available amounts of said urea resins added to the vinyl polymers are within the range from about half the amount to 10 times the amount of the latter.

50

In case other aminoplasts, such as melamine resins, are employed, no permanent hardening effect is obtained through such effect is displayed at the initial stage, and therefore it is hardly possible to attain the object of the present invention.

55

In carrying out the process of the present invention, the fabric as above-identified is soaked in an aqueous solution containing the vinyl polymer and, if desired, the aminoplast, as above-mentioned, along with magnesium chloride, and then the soaked fabric is subjected to the conventional procedures which are known in the general resin-finishing processes. For example, the fabric is squeezed by means of rolls or a mangle, or by means of centrifugation, and then dried at a temperature below 105° C. Thereafter the fabric is cured by heat-treatment at a temperature of 110° to 200° C., preferably 120° to 160° C., for a few seconds to about 10 minutes, then washed with an alkaline solution to remove the residual acid in the fabric, and then dried.

60

The fabrics which are advantageously processed according to the invention include those of such synthetic hydrophobic fibers, as polyester, polyacrylic, and partially acetylated cellulose fibers. The typical polyester is polyethylene terephthalate and its analogs. The polyacrylic fibers include those made of acrylonitrile polymer and

65

70

75

copolymers containing a major part of acrylonitrile. The partially acetylated cellulose fibers include those obtained from cellulose acetylated in various degree or those obtained by after-acetylation of cellulose fibers.

In the following, the present invention will be illustrated with reference to examples.

subjected to the same saponification as in the case of "resin B" to obtain a resin (molecular weight: about 22,000), which was then dissolved in water to form a 15% paste. This paste was referred to as "resin C."

By use of said resins A, B and C, the following 12 kinds of resin baths were prepared:

| Resin baths | Components               |                                             |                                                |                                                       |                               |
|-------------|--------------------------|---------------------------------------------|------------------------------------------------|-------------------------------------------------------|-------------------------------|
|             | Resins (part)<br>Resin A | Dimethoxy-methyluron (part of 50% aq. sol.) | Dimethylol ethyleneurea (part of 50% aq. sol.) | Dimethylol glyoxal mono-ureine (part of 50% aq. sol.) | 30% magnesium chloride (part) |
| A           | 10                       |                                             |                                                |                                                       | 3                             |
| A-1         | 7.5                      | 8                                           |                                                |                                                       | 4.5                           |
| A-2         | 7.5                      |                                             | 8                                              |                                                       | 3.8                           |
| A-3         | 7.5                      |                                             |                                                | 8                                                     | 4.5                           |
| Resin B     |                          |                                             |                                                |                                                       |                               |
| B           | 10                       |                                             |                                                |                                                       | 3                             |
| B-1         | 7.5                      | 8                                           |                                                |                                                       | 4.5                           |
| B-2         | 7.5                      |                                             | 8                                              |                                                       | 3.8                           |
| B-3         | 7.5                      |                                             |                                                | 8                                                     | 4.5                           |
| Resin C     |                          |                                             |                                                |                                                       |                               |
| C           | 10                       |                                             |                                                |                                                       | 3                             |
| C-1         | 7.5                      | 8                                           |                                                |                                                       | 4.5                           |
| C-2         | 7.5                      |                                             | 8                                              |                                                       | 3.8                           |
| C-3         | 7.5                      |                                             |                                                | 8                                                     | 4.8                           |

NOTE.—The volume of each bath was made 100 cc. by addition of water.

Vinyl polymers were obtained according to the following processes:

#### Resin A

40

172 parts of vinyl acetate and 32 parts of acrolein diacetate were dispersed in 320 parts of water together with 0.1 part of polyvinyl alcohol (a dispersing agent). To the resulting dispersion, 0.2 part of benzoyl peroxide was added, and the mixture was allowed to polymerize for 5 hours at 70° C. The granular polymer yielded was separated, dried and then dissolved in methanol so as to form a 20% solution. 18 parts of caustic soda was added to the solution and the saponification was effected for 2 hours at 35° C. The precipitated white powdery resin (molecular weight: about 200,000) was separated from the methanol by filtration and then dissolved in water to form a 15% paste. This paste was referred to as "resin A."

#### Resin B

45

To a mixture comprising 150 parts of vinyl acetate, 54 parts of acrolein diacetate, and 44 parts of methanol, there was added 0.2 part of benzoyl peroxide. After 48 hours polymerization under stirring at 60° C., the reaction mass was mixed with 750 parts of methanol and 10 parts of caustic soda and saponified for 2 hours at 40° C. The resulting white powdery resin (molecular weight: 73,000) was separated and dissolved in water to yield a 15% paste. This paste was referred to as "resin B."

#### Resin C

50

To a mixture comprising 13 parts of acrolein, 237 parts of vinyl acetate and 62 parts of methanol, there was added 7.5 parts of  $\alpha,\alpha'$ -azobisisobutyronitrile, and the mixture was allowed to polymerize with agitation at 60° C. for 20 hours. The resulting polymerizate was

Subsequently, partially after-acetylated cellulose fiber fabrics muslin and a mix-spun broad of polyethylene terephthalate fibers and cotton were immersed in each of these baths, squeezed by means of a mangle, dried at 80° C. for 2 minutes, heat-treated at 140° C. for 4 minutes, washed with an alkaline cleanser and then dried.

The hardening and soil resistance were as shown in the following tables.

TABLE 3.—RESULTS OF TESTS WITH PARTIALLY ACETYLATED CELLULOSE MUSLIN

| Processing                                       | Bending length before washing <sup>1</sup> (warp and weft) (mm.) | Bending length after washing (warp and weft) (mm.) |
|--------------------------------------------------|------------------------------------------------------------------|----------------------------------------------------|
| Non-processed cloth                              | 65                                                               | 62                                                 |
| Resin bath:                                      |                                                                  |                                                    |
| A                                                | 130                                                              | 107                                                |
| A-1                                              | 146                                                              | 132                                                |
| A-2                                              | 135                                                              | 114                                                |
| A-3                                              | 141                                                              | 121                                                |
| B                                                | 125                                                              | 100                                                |
| B-1                                              | 139                                                              | 130                                                |
| B-2                                              | 129                                                              | 114                                                |
| B-3                                              | 141                                                              | 120                                                |
| C                                                | 119                                                              | 97                                                 |
| C-1                                              | 137                                                              | 128                                                |
| C-2                                              | 124                                                              | 115                                                |
| C-3                                              | 133                                                              | 120                                                |
| A methylated trimethylolamine paste <sup>2</sup> | 110                                                              | 70                                                 |
| P.V.A. <sup>3</sup>                              | 112                                                              | 69                                                 |

<sup>1</sup> Washing was repeated 5 times according to home-washing process by means of an agitation-type electric washing machine.

<sup>2</sup> The bath shown in the table was prepared by dissolving 5 parts of this resin paste and 0.5 part of 30% 2-amino-2-methylpropanol hydrochloride in water to make the volume of the resulting solution 100 cc.

<sup>3</sup> The P.V.A. bath was prepared by dissolving 1.5 parts of polyvinyl alcohol to make the volume of the resulting solution 100 cc.

TABLE 4.—RESULTS OF TESTS WITH A MIX-SPUN FABRIC OF A POLYETHYLENE TEREPHTHALATE FIBER WITH COTTON

| Processing                                           | Bending length before washing (warp and weft) (mm.) | Bending length after washing (warp and weft) (mm.) | Dirt test (naked eyes)      |                            | Dirt test <sup>1</sup> (brightness) |                            |
|------------------------------------------------------|-----------------------------------------------------|----------------------------------------------------|-----------------------------|----------------------------|-------------------------------------|----------------------------|
|                                                      |                                                     |                                                    | Before washing <sup>2</sup> | After washing <sup>2</sup> | Before washing <sup>2</sup>         | After washing <sup>2</sup> |
| Non-processed cloth                                  | 76                                                  | 72                                                 | X                           | X                          | 35                                  | 34                         |
| Resin bath:                                          |                                                     |                                                    |                             |                            |                                     |                            |
| A                                                    | 100                                                 | 90                                                 | 0                           | 0                          | 61                                  | 53                         |
| A-1                                                  | 121                                                 | 115                                                | 0                           | 0                          | 64                                  | 58                         |
| A-2                                                  | 110                                                 | 103                                                | 0                           | 0                          | 55                                  | 49                         |
| A-3                                                  | 118                                                 | 113                                                | 0                           | 0                          | 59                                  | 54                         |
| B                                                    | 98                                                  | 89                                                 | 0                           | 0                          | 59                                  | 51                         |
| B-1                                                  | 111                                                 | 104                                                | 0                           | 0                          | 61                                  | 56                         |
| B-2                                                  | 107                                                 | 99                                                 | 0                           | 0                          | 55                                  | 49                         |
| B-3                                                  | 112                                                 | 106                                                | 0                           | 0                          | 59                                  | 52                         |
| C                                                    | 95                                                  | 88                                                 | 0                           | 0                          | 58                                  | 50                         |
| C-1                                                  | 109                                                 | 103                                                | 0                           | 0                          | 59                                  | 55                         |
| C-2                                                  | 102                                                 | 96                                                 | 0                           | 0                          | 54                                  | 50                         |
| C-3                                                  | 107                                                 | 101                                                | 0                           | 0                          | 59                                  | 51                         |
| A methylated trimethylolmelamine paste. <sup>3</sup> | 90                                                  | 77                                                 | Δ                           | X                          | 43                                  | 37                         |
| P.V.A. <sup>4</sup>                                  | 89                                                  | 77                                                 | Δ                           | X                          | 42                                  | 36                         |

<sup>1</sup> The brightness was determined by measurement of reflexing ratio at 550 m $\mu$ , based upon magnesium oxide white, by use of Recording Spectrophotometer made by General Electric Co.

<sup>2</sup> Each dirt test was carried out by putting a test cloth (5 cm. x 5 cm.) in a Leunder-O-meter containing the following dirtying bath at a bath ratio of 1:50, taking out the cloth after one minute's operation, washing the cloth with water, drying, and then judging the dirtiness degree by naked eyes. The dirtying bath was prepared by dissolving in 250 cc. of carbon tetrachloride, 1 g. of carbon black, 0.5 g. of beef tallow and 2 g. of liquid paraffin.

<sup>3</sup> The bath shown in the table was prepared by dissolving 5 parts of this resin paste and 0.5 part of 30% 2-amino-2-methylpropanol hydrochloride in water to make the volume of the resulting solution 100 cc.

<sup>4</sup> The P.V.A. bath was prepared by dissolving 1.5 parts of polyvinyl alcohol to make the volume of the resulting solution 100 cc.

0—scarcely made dirty. Δ—somewhat made dirty. X—made dirty.

Furthermore, the effectivenesses of the combined use of the various aminoplasts according to the invention are set forth in the following Table 5.

TABLE 5.—EFFECTIVENESSES OF THE COMBINED USE OF VARIOUS AMINOPLASTS (A MIXED SPUN POLYETHYLENE TEREPHTHALATE-COTTON BROADCLOTH).

| Resin A (part)       | Components                        |                              | Bending length (warp and weft, mm.) |               |
|----------------------|-----------------------------------|------------------------------|-------------------------------------|---------------|
|                      | 50% aminoplasts (part)            | 30% MgCl <sub>2</sub> (part) | Before washing                      | After washing |
| 10                   |                                   | 3                            | 105                                 | 96            |
| 10                   | Dimethylolethyleneurea (8).       | 4.6                          | 130                                 | 108           |
| 10                   | Dimethoxymethyl-ethylenurea (8).  | 4.6                          | 136                                 | 110           |
| 10                   | Dimethyloluron (8).               | 5.5                          | 138                                 | 122           |
| 10                   | Dimethoxymethyl-uron (8).         | 5.5                          | 143                                 | 129           |
| 10                   | Tetramethylolacetylenediurea (8). | 5.5                          | 130                                 | 115           |
| 10                   | Dimethylolmethyl-triazone (8).    | 4.6                          | 125                                 | 106           |
| Non-processed cloth. |                                   |                              | 80                                  | 77            |

What we claim is:

1. A resin composition used for the processing of fabrics comprising fibers selected from the group consisting of polyester, polyacrylic and partially acetylated cellulosic fibers to endow them with permanent soil resistance and hardness, which consists essentially of an aqueous solution of a water soluble vinyl polymer containing hydroxyl and aldehyde groups in the molecule which is obtained by saponification of a copolymer of vinyl acetate with vinyl acetate with a member selected from the group consisting of acrolein and acrolein diacetate, said aqueous solution containing magnesium chloride as catalyst.

2. A resin composition used for the processing of fabrics comprising fibers selected from the group consisting of polyester, polyacrylic and partially acetylated cellulosic fibers to endow them with permanent soil resistance and hardness, which consists essentially of an aqueous solution of a water soluble vinyl polymer containing hydroxyl and aldehyde groups in the molecule which is obtained

30 by saponification of a copolymer of vinyl acetate with a member selected from the group consisting of acrolein and acrolein diacetate, said aqueous solution containing magnesium chloride as catalyst.

35 3. A process for imparting permanent soil resistance and hardness to fabrics comprising fibers selected from the group consisting of polyester, polyacrylic and partially acetylated cellulosic fibers, which comprises soaking said fabric in a resin bath consisting essentially of an aqueous solution of a water soluble vinyl polymer containing hydroxyl and a aldehyde groups in the molecule, which is obtained by saponification of a copolymer of vinyl acetate with a member selected from the group consisting of acrolein and acrolein diacetate, said aqueous solution being added with magnesium chloride as catalyst.

40 4. A process for imparting permanent soil resistance and hardness to fabrics comprising fibers selected from the group consisting of polyester, polyacrylic and partially acetylated cellulosic fibers, which comprises soaking said fabric in a resin bath consisting essentially of an aqueous solution of a water soluble vinyl polymer and at least one aminoplast, said vinyl polymer containing hydroxyl and aldehyde groups in the molecule, which is obtained by saponification of a copolymer of vinyl acetate with a member selected from the group consisting of acrolein and acrolein diacetate, said aminoplast being a member selected from the group consisting of dimethylolethyleneurea, dimethyloluron, dimethylolgly-

45 oxalmonourein, tetramethylolacetylenediurea, dimethyloltriazone and their alkylated derivatives.

50 5. A process for imparting permanent soil resistance and hardness to fabrics comprising fibers selected from the group consisting of polyester, polyacrylic and partially acetylated cellulosic fibers, which comprises soaking said fabric in a resin bath consisting essentially of an aqueous solution of a water soluble vinyl polymer and at least one aminoplast, said vinyl polymer containing hydroxyl and aldehyde groups in the molecule, which is obtained by saponification of a copolymer of vinyl acetate with a member selected from the group consisting of acrolein and acrolein diacetate, said aminoplast being a member selected from the group consisting of dimethylolethyleneurea, dimethyloluron, dimethylolgly-

55 oxalmonourein, tetramethylolacetylenediurea, dimethyloltriazone and their alkylated derivatives, and said aqueous solution being added with magnesium chloride as catalyst.

#### References Cited by the Examiner

#### UNITED STATES PATENTS

|           |         |               |         |
|-----------|---------|---------------|---------|
| 2,485,239 | 10/1949 | Izard         | 260—73  |
| 2,569,932 | 10/1951 | Izard         | 260—73  |
| 2,950,553 | 8/1960  | Hurwitz       | 117—143 |
| 3,149,999 | 9/1964  | Enders et al. | 117—161 |

MURRAY TILLMAN, Primary Examiner.

JAMES A. SEIDLECK, Examiner.

E. J. TROJNAR, J. C. BLEUTGE, Assistant Examiners.